

# United States Patent Office

2,728,666

Patented Dec. 27, 1955

1

2,728,666

## STABILIZATION OF EMULSIONS SENSITIZED WITH ALKYLENE OXIDE POLYMERS

Burt H. Carroll, Rochester, N. Y., assignor to Eastman Kodak Company, Rochester, N. Y., a corporation of New Jersey

No Drawing. Application November 8, 1952,  
Serial No. 319,614

24 Claims. (Cl. 95—7)

This invention relates to fog-inhibiting agents and stabilizers for photographic emulsions and to photographic emulsions containing them.

It is known that photographic emulsions, particularly ultra-sensitive emulsions or those containing optical sensitizers exhibit a tendency to form a deposit of silver in the emulsion upon development. This deposit extends more or less uniformly over the entire emulsion and is known as fog. Photographic fog is of two types: local and general. Local fog is formed by exposure of the film or plate at undesired points as by a light leak in the camera. General fog is formed in a number of ways. It may be caused by the conditions of high temperature or humidity or unusually long time of storage. The nature of the emulsion may also produce chemical fog as well as the conditions of development of the emulsion as by development for protracted periods of time or at temperatures above normal. We are primarily concerned with fog and sensitivity changes in photographic films produced by storage under adverse conditions of temperature and humidity or for prolonged periods of time before exposure and development.

General fog and loss of sensitivity of the emulsion are especially likely to occur when the sensitive material is stored under conditions other than ideal, that is, under conditions of high temperature and humidity, as in tropical regions.

It is known that the effective sensitivity of photographic silver halide emulsions may be increased by adding to them derivatives of alkylene oxides such as ethylene oxide polymers having molecular weights of 300 or more. The practical value of these compounds is severely limited by their tendency to increase fog on storage of the photographic film, especially storage at elevated temperatures and humidities. It has been found difficult to control this by the antifoggants commonly available without using quantities of antifog that partly neutralize the speed increase obtained from the alkylene oxide derivatives.

It is therefore an object of the present invention to provide a method for stabilizing photographic emulsions sensitized with alkylene oxide derivatives such as polyethylene oxides. A further object is to provide a means for reducing the fog produced upon keeping of emulsions so sensitized, especially emulsions stored under tropical or other adverse conditions. A still further object is to provide a means for stabilizing the speed and contrast of emulsions so sensitized. Other objects will appear from the following description of my invention.

These objects are accomplished in general by adding to the emulsion sensitized with alkylene oxide polymers, certain organic compounds of mercury in which the mercury atom has at least one ionizable bond, or simple mercuric or mercurous salts of an inorganic or organic acid.

The alkylene oxide polymers used to sensitize the emulsions may be of various types. The alkylene oxides from which the polymers are derived contain from 2 to 4 carbon atoms, e. g., ethylene oxide, propylene oxide and

2

butylene oxide. The preparation of polymers from these compounds is described in Ellis, *The Chemistry of Synthetic Resins* (1935), pages 990 to 994. These compounds are also referred to as polyalkylene glycols and their use as sensitizers for silver halide emulsions is described in U. S. Patents 2,423,549 and 2,441,389.

Various derivatives of alkylene oxides may also be used to sensitize the silver halide emulsions, e. g., condensation products of alkylene oxide with glycols, such as those having from 8 to 18 carbon atoms as described in U. S. Patent 2,240,472 and British Patent 443,559, as well as condensation products of alkylene oxides with aliphatic alcohols, aliphatic acids and aliphatic amines, that is, polyalkylene ethers, esters and amides, the preparation of which is described in U. S. Patent 1,970,578, and condensation products of alkylene oxides with hexitol ring dehydration products, as described in U. S. Patent 2,400,532.

In each case the polyalkylene oxide or derivative of alkylene oxide should have a molecular weight of at least 300 and preferably a molecular weight of 1500 to 4000 or more.

The compounds of mercury used to stabilize emulsions sensitized with the polyalkylene oxides are of three types: (1) molecular compounds of mercuric salts with amines or salts of amines, (2) organic compounds of mercury in which the mercury atom is attached by a non-ionic or covalent bond to an organic nucleous, especially a heterocyclic organic nucleus, and by an ionic or electrovalent bond to an anion, and (3) simple salts of mercury with organic or inorganic acids.

The principal purpose of my invention is to provide a means for maintaining the sensitivity and fog of silver halide emulsions at or close to initial optimum values under keeping conditions of high temperature and humidity. Preferably, the fog inhibitors which I propose to use are added to the emulsion at any stage during the process of manufacture prior to coating the emulsion. The mercury fog inhibitor may be added to the emulsion in solution in any convenient solvent not injurious to the emulsion such as water, lower alcohols and ketones.

A solution of the mercuric compound which I employ when added in suitable concentration before coating to unsensitized or optically sensitized silver halide emulsions usually does not appreciably affect the sensitivity and fog when measurements are made soon after coating. However, when sensitometric measurements are made after appreciable intervals of time under tropical or dry conditions of storage at elevated temperatures, these compounds do stabilize speed and maintain fog at a low level.

Any of the mercuric compounds disclosed in Allen, Byers and Murray U. S. application Serial No. 319,611, filed concurrently herewith, may be used to stabilize the emulsions according to my invention. The following is typical:



Bis(2-amino-5-iodopyridine hydroiodide) mercuric iodide

Any of the mercuric compounds disclosed in Leubner and Murray U. S. application Serial No. 319,613, filed concurrently herewith, may also be used. The following is typical:



2-pyridyl mercuric chloride

Any of the compounds disclosed in Carroll and Murray U. S. application Serial No. 319,612, filed concurrently herewith may also be used. These compounds include mercuric and mercurous chloride, bromide and iodide, mercuric acetate, mercuric nitrate, mercurous sulfate, etc.

The alkylene oxide derivatives used to sensitize the emulsions may be illustrated by the following specific examples, although my invention is in no way limited to the use of these specific compounds.



where  $n$ =an integer greater than about 10.

The preparation of silver halide emulsions involves three separate operations: (1) the emulsification and digestion or ripening of the silver halide, (2) the freeing of the emulsion from aqueous soluble salts usually by washing, (3) the second digestion or after-ripening to obtain increased sensitivity (Mees, *The Theory of the Photographic Process*, 1942, page 3). The fog inhibiting agents may be added at any stage, e. g., after the final digestion.

The photographic emulsions which I use are of the developing-out type and best results have been obtained with gelatino-silver bromoiodide emulsions. However, emulsions of varying halide content may be used.

The emulsions may be chemically sensitized by any of the accepted procedures, in addition to or in combination with the sensitizing with alkylene oxide polymers. The emulsions may be digested with naturally active gelatin, or sulfur compounds may be added such as those described in Sheppard U. S. Patent 1,574,944 and 1,623,499, and Sheppard and Brigham U. S. Patent 2,410,689.

The emulsions may also be treated with salts of the noble metals such as ruthenium, rhodium, palladium, iridium and platinum, all of which belong to group VIII of the periodic table of elements and have an atomic weight greater than 100. Representative compounds are ammonium chloropalladate, potassium chloroplatinate and sodium chloropalladate, which are used for sensitizing in amounts below that which produces any substantial fog inhibition, as described in Smith and Trivelli U. S. Patent 2,448,060, and as antifoggants in higher amounts, as described in Trivelli and Smith U. S. Patents 2,566,245 and 2,566,263.

The emulsions may also be chemically sensitized with gold salts as described in Waller and Dodd U. S. Patent 2,399,083, Damschroder U. S. Patent 2,597,856, and Yutzy and Leermakers U. S. Patent 2,597,915. Suitable compounds are potassium chloroaurite, potassium aurithiocyanate, potassium chloroaurate, auric trichloride and 2-aurosulfonylbenzothiazole methochloride.

The emulsions may also be chemically sensitized with reducing agents such as stannous salts (Carroll U. S. Patent 2,487,850), polyamines such as diethylene triamine (Lowe and Jones U. S. Patent 2,518,698), polyamines such as spermine (Lowe and Allen U. S. Patent

2,521,925), or bis-( $\beta$ -aminoethyl) sulfide and its water-soluble salts (Lowe and Jones U. S. Patent 2,521,926).

The sensitizing and stabilizing combinations of polyalkylene oxides and the mercuric compounds are effective in the presence or absence of optical sensitizing dyes. Since optical sensitizing may affect stability of emulsions with respect to sensitivity, fog and latent image changes, the action of the compounds of this invention is not completely independent of optical sensitizing or other emulsion variables. I have found, however, that both unsensitized emulsions and emulsions sensitized with cyanine or merocyanine dyes or both may be treated with polyalkylene oxides and mercuric compounds according to my invention.

15 The most useful concentration of the mercuric compound in the emulsion is from about 0.05 mg. to 1.0 mg. per gram mole of silver halide in the emulsion. Although higher amounts may be used, I have found that no emulsion is likely to tolerate as much as 5 times this 20 upper limit without serious desensitization. Optimum concentrations are about 0.5 mg. per gram mole of silver halide for the molecular compounds of mercuric salts with amines or salts of amines, about 0.1 mg. per gram mole of silver halide for the organic compounds of mercury in which the mercury atom is attached by a non-ionic bond to an organic nucleus and by an ionic bond to an anion, and from 0.05 mg. to 0.5 mg. for the simple mercuric salts such as mercuric chloride and mercuric iodide.

25 30 The stabilizing action was determined by incubation of the emulsions, usually for one week at 120° F. and 20% relative humidity, unless otherwise stated in the examples. The results of aging tests are tabulated below and compare speed, gamma and fog of the emulsions with 35 and without the stabilizing compound.

#### Example I

One liter of a negative speed gelatino-silver bromoiodide emulsion containing 0.24 mole of silver halide per liter was digested with a sulfur compound such as disclosed in Sheppard U. S. Patent 1,574,944 and potassium chloroaurate and optically sensitized in the conventional manner. To a portion of the emulsion there was added 52.5 grams per gram mole of silver halide of a polyethylene oxide having a molecular weight of 300, and to a portion of this emulsion there was also added 0.7 mg. per gram mole of silver halide of bis-(2-amino-5-iodopyridine hydroiodide) mercuric iodide.

50 The emulsions were coated on film base and were exposed on an Eastman type Ib Sensitometer and developed for 8 minutes at 68° F. in a developer of the following formula:

|                                | Grams |
|--------------------------------|-------|
| N-methyl-p-aminophenol sulfate | 1.5   |
| 55 Hydroquinone                | 1.3   |
| Sodium sulfite (desiccated)    | 75    |
| Borax                          | 4.5   |
| Potassium bromide              | 0.4   |
| Water to 1 liter.              |       |

60 The films with and without the various addenda were held at 120° F. and 20% relative humidity for one week and were then exposed and developed as indicated. The results of tests for speed, gamma and fog were as follows:

| Compound                                                    | Agent per mole, gm. | Fresh Test |       |     | After Incubation |       |     |
|-------------------------------------------------------------|---------------------|------------|-------|-----|------------------|-------|-----|
|                                                             |                     | Speed      | Gamma | Fog | Speed            | Gamma | Fog |
| (I) Polyethylene glycol 300                                 | 52.5                | 1,320      | 1.41  | .09 | 2,200            | 1.21  | .47 |
| I+ Bis-(2-amino-5-iodopyridine hydroiodide) mercuric iodide | 0.7                 | 1,100      | 1.31  | .06 | 2,150            | 1.44  | .21 |

## Example 2

One liter of a gelatino-silver bromoiodide emulsion with a sulfur compound such as disclosed in Sheppard U. S. Patent 1,574,944 and potassium chloroaurate, and optically sensitized with a mixture of cyanine dyes in the conventional way. To portions of the emulsion the mercuric compound bis-(2-amino-5-iodopyridine hydroiodide)mercuric iodide was added in varying amounts and to other portions of the emulsion the mercuric compound was added together with the condensation product of 1 mole of oleyl alcohol with approximately 25 moles of ethylene oxide. Upon incubation of samples of the emulsions as indicated in the table, and measurement of speeds as 30/E where E is the exposure in meter-candle-seconds of approximately sunlight distribution required to produce a density of 0.20 above fog, the following results were obtained upon development for 6.5 minutes in

emulsion was divided into several portions and to some of these were added a polyethylene oxide having a molecular weight of about 4000 (Carbowax 4000), and the mercuric compounds shown in the table below. Each of these emulsions was coated and the coatings were exposed on a Jb sensitometer and developed for three minutes in a developer of the following composition:

|                                | Grams |
|--------------------------------|-------|
| N-methyl-p-aminophenol sulfate | 2.2   |
| 10 Hydroquinone                | 8.8   |
| Sodium sulfite (desiccated)    | 96    |
| Sodium carbonate, monohydrate  | 56    |
| Potassium bromide              | 5     |
| Water to 1 liter.              |       |

Upon testing for speed, gamma and fog, before and after incubation as in Example 1, the following results were obtained:

| Compound                                            | mg./mole | Fresh Test |       |     | After Incubation |       |     |
|-----------------------------------------------------|----------|------------|-------|-----|------------------|-------|-----|
|                                                     |          | Speed      | Gamma | Fog | Speed            | Gamma | Fog |
| Control                                             |          | 165        | 1.38  | .07 | 165              | 1.27  | .10 |
| (I) With Carbowax 4000                              | 600      | 280        | 1.34  | .10 | 240              | 1.34  | .14 |
| I+ (2-amino-5-iodopyridine)·<br>HI-HgI <sub>2</sub> | 0.6      | 235        | 1.36  | .09 | 210              | 1.43  | .11 |
| I+ Mercuric chloride                                | .06      | 235        | 1.40  | .10 | 240              | 1.35  | .12 |
| Do                                                  | .15      | 215        | 1.39  | .09 | 220              | 1.39  | .12 |
| I+ Pyridyl mercuric chloride                        | 0.6      | 205        | 1.34  | .10 | 220              | 1.39  | .12 |

a developer of the following composition:

|                                |       |     |
|--------------------------------|-------|-----|
| Water                          | cc    | 750 |
| N-methyl-p-aminophenol sulfate | grams | 2   |
| Hydroquinone                   | do    | 5   |
| Sodium sulfite (desiccated)    | do    | 35  |
| Borax (granular)               | do    | 100 |
| Water to 1 liter.              |       | 2   |

## Example 4

A medium speed gelatino-silver bromoiodide emulsion was sensitized with a mixture of gold and sulfur compounds as in Example 2, and divided into two portions. To one portion of this emulsion there was added a mixture of the reduction sensitizer triethylene tetramine (U. S. Patent 2,518,698) and a polyethylene oxide hav-

| Compound                                                      | mg./mole | Original Sensitivity |       |      | Sensitivity after 1 week at 100° F. in packages sealed at 74° F., 54% RH |       |      |
|---------------------------------------------------------------|----------|----------------------|-------|------|--------------------------------------------------------------------------|-------|------|
|                                                               |          | Speed                | Gamma | Fog  | Speed                                                                    | Gamma | Fog  |
| Control                                                       |          | 7,050                | 0.82  | 0.10 | 7,050                                                                    | 0.75  | 0.12 |
| (A) Bis(2-amino-5-iodopyridine hydroiodide)mercuric iodide    | 0.56     | 7,200                | 0.70  | 0.09 | 7,350                                                                    | 0.75  | 0.11 |
| Do                                                            | 0.80     | 6,900                | 0.79  | 0.09 | 4,850                                                                    | 0.75  | 0.10 |
| Do                                                            | 1.1      | 6,700                | 0.67  | 0.08 | 7,200                                                                    | 0.76  | 0.08 |
| Control                                                       |          | 7,200                | 0.70  | 0.10 | 6,700                                                                    | 0.71  | 0.13 |
| (B) Condensation product of oleyl alcohol with ethylene oxide | 280      | 11,100               | 0.78  | 0.12 | 8,050                                                                    | 0.75  | 0.26 |
| B 280 mg. + A                                                 | 0.56     | 10,200               | 0.76  | 0.12 | 11,700                                                                   | 0.78  | 0.14 |
| B 280 mg. + A                                                 | 0.80     | 10,200               | 0.73  | 0.12 | 12,800                                                                   | 0.72  | 0.13 |
| B 280 mg. + A                                                 | 1.1      | 10,400               | 0.80  | 0.10 | 12,800                                                                   | 0.85  | 0.10 |

## Example 3

A medium speed gelatino-silver bromoiodide emulsion was sensitized with a mixture of gold and sulfur compounds as in Example 2, and was then digested to optimum speed in the presence of a reduction sensitizer of the type disclosed in my U. S. Patent 2,487,850. This

ing a molecular weight of about 4000 (Carbowax 4000). To separate portions of the emulsion sensitized in this way, there were added the mercuric compounds shown in the table below. Each of these emulsions was exposed, developed and tested as in Example 3, with the following results:

| Compound                                            | mg./mole | Fresh Test |       |     | After Incubation |       |     |
|-----------------------------------------------------|----------|------------|-------|-----|------------------|-------|-----|
|                                                     |          | Speed      | Gamma | Fog | Speed            | Gamma | Fog |
| Control                                             |          | 250        | 1.46  | .09 | 265              | 1.46  | .12 |
| (I) With:                                           |          |            |       |     |                  |       |     |
| Triethylene tetramine                               | 36       |            |       |     |                  |       |     |
| Carbowax 4000                                       | 600      |            |       |     |                  |       |     |
| I+ (2-amino-5-iodopyridine)·<br>HI-HgI <sub>2</sub> | 0.3      | 460        | 1.80  | .18 | 440              | 1.36  | .55 |
| Do                                                  | 1.2      | 235        | 1.92  | .10 | 315              | 1.60  | .09 |
| I+ Mercuric chloride                                | .12      | 370        | 1.91  | .14 | 530              | 1.87  | .34 |
| I+ Pyridyl mercuric chloride                        | 0.6      | 400        | 1.87  | .16 | 540              | 1.29  | .32 |
| Control                                             |          | 240        | 1.55  | .11 | 310              | 1.36  | .14 |

## Example 5

A negative-speed gelatino-silver bromoiodide emulsion was chemically sensitized with sulfur and gold sensitizers as in Example 2 and was digested to optimum speed and divided into two portions. To one portion of this emulsion there was added a polyethylene oxide having a molecular weight of about 4000 (Carbowax 4000). To separate portions of the emulsion sensitized in this way, there were added the mercuric compounds shown in the table below. Each of the emulsions was exposed on a 10 Ib sensitometer and developed for 5 minutes in a developer of the following composition:

| Compound                           | mg./mole | Fresh Test |       |      | After Incubation |       |      |
|------------------------------------|----------|------------|-------|------|------------------|-------|------|
|                                    |          | Speed      | Gamma | Fog  | Speed            | Gamma | Fog  |
| Control                            |          | 3,500      | 0.73  | 0.01 | 2,550            | 0.68  | 0.10 |
| Polyethylene glycol oleyl ether    | 500      | 4,750      | 0.73  | 0.01 | 5,100            | 0.76  | 0.06 |
| K <sub>2</sub> Hg(CN) <sub>4</sub> | 0.125    |            |       |      |                  |       |      |
| Polyethylene glycol oleyl ether    | 500      | 4,350      | 0.77  | 0.02 | 5,100            | 0.75  | 0.02 |
| K <sub>2</sub> Hg(CN) <sub>4</sub> | 0.25     |            |       |      |                  |       |      |
| Polyethylene glycol cetyl ether    | 800      | 4,750      | 0.75  | 0.01 | 5,850            | 0.79  | 0.03 |
| K <sub>2</sub> Hg(CN) <sub>4</sub> | 0.25     |            |       |      |                  |       |      |

|                                | Grams |
|--------------------------------|-------|
| N-methyl-p-aminophenol sulfate | 2.5   |
| Hydroquinone                   | 2.5   |
| Sodium sulfite, desiccated     | 30    |
| Sodium metaborate              | 10    |
| Potassium bromide              | 0.5   |
| Water to 1 liter.              |       |

Samples with and without the various addenda were held at 120° F. and 20% relative humidity for three days and were then exposed and developed as indicated. The results of tests for speed, gamma and fog were as follows:

| Compound                                                  | mg./mole | Fresh Test |       |     | After Incubation |       |     |
|-----------------------------------------------------------|----------|------------|-------|-----|------------------|-------|-----|
|                                                           |          | Speed      | Gamma | Fog | Speed            | Gamma | Fog |
| Control                                                   |          | 5,900      | 0.83  | .08 | 3,000            | 0.89  | .21 |
| (I) With Carbowax 4000                                    | 500      | 8,800      | 0.82  | .08 | 3,800            | 0.75  | .27 |
| I+(2-amino-5-iodopyridine)· <sub>2</sub> HgI <sub>2</sub> | 1.0      | 8,200      | 0.82  | 0.7 | 3,550            | 0.87  | .11 |
| I+Mercuric iodide                                         | .25      | 7,400      | 0.85  | 0.8 | 4,800            | 0.72  | .20 |
| Do                                                        | 1.0      | 6,100      | 0.88  | 0.6 | 3,200            | 0.82  | .06 |

## Example 6

In order to illustrate the action of the mercury anti-foggants on an emulsion containing both a polyethylene oxide and a chloropalladate, an emulsion of the type used in Example 5 was treated with these agents as shown in the table below, and processed as described in Example 5. The following results were obtained:

50 8-chloromercuriquinoline, as shown in the following table. These emulsions were coated on a cellulose acetate support, exposed on a Ib Sensitometer and developed for 3 minutes in a developer having the same composition as that shown in Example 3. Upon incubation of each of the coatings for two weeks at 120° F. and testing

| Compound                                                  | mg./mole | Fresh Test |       |     | After Incubation |       |     |
|-----------------------------------------------------------|----------|------------|-------|-----|------------------|-------|-----|
|                                                           |          | Speed      | Gamma | Fog | Speed            | Gamma | Fog |
| Ammonium chloropalladate                                  | 500      | 3,800      | 0.96  | .10 | 2,950            | 0.84  | .18 |
| (I) date                                                  | 500      | 4,200      | 0.94  | .12 | 3,200            | 0.80  | .20 |
| +Carbowax 4000                                            | 500      |            |       |     |                  |       |     |
| I+(2-amino-5-iodopyridine)· <sub>2</sub> HgI <sub>2</sub> | 1.0      | 3,300      | 0.96  | .12 | 4,150            | 0.72  | .08 |
| I+Mercuric iodide                                         | 0.25     | 2,950      | 1.0   | .10 | 4,750            | 0.74  | .08 |

## Example 7

A negative-speed gelatino-silver bromoiodide emulsion

both sets of coatings for speed, gamma and fog, the following results were obtained:

| Compound                  | mg./mole | Fresh Test |       |     | After Incubation |       |     |
|---------------------------|----------|------------|-------|-----|------------------|-------|-----|
|                           |          | Speed      | Gamma | Fog | Speed            | Gamma | Fog |
| Control                   |          | 400        | 0.89  | .09 | 300              | 0.65  | .38 |
| (I) With Carbowax 4000    | 550      | 470        | 1.13  | .12 | 350              | 0.66  | .55 |
| +8-chloromercuriquinoline | .825     | 390        | 1.21  | .11 | 530              | 0.68  | .23 |
| Do                        | 1.1      | 420        | 1.16  | .11 | 760              | 0.73  | .16 |

Instead of incorporation in the silver halide emulsion the fog-inhibitors of my invention may be incorporated in a colloid layer such as a gelatin layer on one or both sides of the film or they may be incorporated in a processing bath such as a developer or pre-bath.

The fog-inhibiting agents which I have described may be used in various kinds of photographic emulsions. In addition to being useful in ordinary non-sensitized emulsions they may also be used in orthochromatic, panchromatic and X-ray emulsions. If used with sensitizing dyes, they may be added to the emulsion before or after the dyes are added. Various silver salts may be used as the sensitive salt, such as silver bromide, silver iodide, silver chloride or mixed silver halides. The mercury compounds and alkylene oxide polymers may be used in emulsions intended for color photography, for example, emulsions containing color-forming couplers, or emulsions to be developed by solutions containing couplers.

The dispersing agents may be gelatin or other colloid such as collodion, albumen, cellulose derivatives or synthetic resins.

It will be understood that I contemplate as included within my invention all modifications and equivalents falling within the scope of the appended claims.

What I claim is:

1. A light-sensitive silver halide emulsion sensitized with an alkylene oxide polymer selected from the class consisting of (1) polyalkylene glycols, (2) condensation products of alkylene oxide with glycols, (3) condensation products of alkylene oxide with aliphatic compounds selected from the class consisting of alcohols, acids and amines and (4) condensation products of alkylene oxide with hexitol ring dehydration products, said alkylene oxide containing from 2 to 4 carbon atoms and said alkylene oxide polymer having a molecular weight of at least 300, said emulsion containing a small amount of a mercury compound selected from the class consisting of (1) a molecular addition compound of a mercury salt with a nitrogen compound of the class consisting of heterocyclic nitrogen compounds in which at least three bonds of the heterocyclic nitrogen atom are attached to carbon, amine-substituted mononuclear aromatic compounds in which three bonds of the amino nitrogen atom are attached to carbon, their halogen acid salts, and the halogen acid salts of aliphatic amines containing at least three carbon atoms, (2) organic compounds of mercury in which the mercury atom is attached by a non-ionic mercury to carbon bond to a cyclic organic nucleus and by an ionic bond to an anion, and (3) simple salts of mercury with organic and inorganic acids.

2. A light-sensitive silver halide emulsion sensitized with an ethylene oxide polymer having a molecular weight of at least 300, said emulsion containing a small amount of a molecular compound of a mercuric salt with a halogen acid salt of a primary amine substituted heterocyclic nitrogen compound.

3. A light-sensitive silver halide emulsion sensitized with an ethylene oxide polymer having a molecular weight of at least 300, said emulsion containing a small amount of an organic compound of mercury in which the mercury atom is attached by a nonionic mercury to carbon bond to a cyclic organic nucleus and by an ionic bond to an anion.

4. A light-sensitive silver halide emulsion sensitized with an ethylene oxide polymer having a molecular weight of at least 300, said emulsion containing a small amount of a simple salt of mercury with an inorganic acid.

5. A light-sensitive silver halide emulsion sensitized with a polyethylene glycol having a molecular weight of at least 300, said emulsion containing a small amount of a molecular compound of a mercuric salt with a halogen acid salt of a primary amine substituted heterocyclic nitrogen compound.

6. A light-sensitive silver halide emulsion sensitized

with a polyethylene glycol having a molecular weight of at least 300, said emulsion containing a small amount of an organic compound of mercury in which the mercury atom is attached by a non-ionic mercury to carbon bond to a cyclic organic nucleus and by an ionic bond to an anion.

7. A light-sensitive silver halide emulsion sensitized with a polyethylene glycol having a molecular weight of at least 300, said emulsion containing a small amount of a simple salt of mercury with an inorganic acid.

8. A light-sensitive sulfur sensitized silver halide emulsion additionally sensitized with an ethylene oxide polymer selected from the class consisting of (1) polyethylene glycols, (2) condensation products of ethylene oxide with glycols, (3) condensation products of ethylene oxide with aliphatic compounds selected from the class consisting of alcohols, acids and amines, and (4) condensation products of ethylene oxide with hexitol ring dehydration products, said ethylene oxide polymer having a molecular weight of at least 300, said emulsion containing a small amount of a mercury compound selected from the class consisting of (1) a molecular addition compound of a mercury salt with a nitrogen compound of the class consisting of heterocyclic nitrogen compounds in which at least three bonds of the heterocyclic nitrogen atom are attached to carbon, amine-substituted mononuclear aromatic compounds in which three bonds of the amino nitrogen atom are attached to carbon, their halogen acid salts, and the halogen acid salts of aliphatic amines containing at least three carbon atoms, (2) organic compounds of mercury in which the mercury atom is attached by a non-ionic mercury to carbon bond to a cyclic organic nucleus and by an ionic bond to an anion, and (3) simple salts of mercury with organic and inorganic acids.

9. A light-sensitive sulfur sensitized gelatino-silver halide emulsion additionally sensitized with a polyethylene glycol having a molecular weight of at least 300, said emulsion containing a small amount of a molecular compound of a mercuric salt with a halogen acid salt of a primary amine substituted heterocyclic nitrogen compound.

10. A light-sensitive sulfur sensitized gelatino-silver halide emulsion additionally sensitized with a polyethylene glycol having a molecular weight of at least 300, said emulsion containing a small amount of a molecular compound of bis-(2-amino-5-iodopyridine)-hydroiodide mercuric halide.

11. A light-sensitive sulfur sensitized gelatino-silver halide emulsion additionally sensitized with a polyethylene glycol having a molecular weight of at least 300, said emulsion containing a small amount of an organic compound of mercury in which the mercury atom is attached by a non-ionic mercury to carbon bond to a cyclic organic nucleus and by an ionic bond to an anion.

12. A light-sensitive sulfur sensitized gelatino-silver halide emulsion additionally sensitized with a polyethylene glycol having a molecular weight of at least 300, said emulsion containing a small amount of a simple salt of mercury with an inorganic acid.

13. A light-sensitive sulfur sensitized gelatino-silver halide emulsion additionally sensitized with polyethylene glycol oleyl ether and containing a small amount of a molecular compound of a mercuric halide with a halogen acid salt of a primary amine substituted heterocyclic nitrogen compound.

14. A light-sensitive sulfur sensitized gelatino-silver halide emulsion additionally sensitized with a polyethylene glycol having a molecular weight of approximately 4000, said emulsion containing a small amount of a bis-(2-amino-5-iodopyridine) hydroiodide mercuric halide.

15. The emulsion of claim 8 which is additionally chemically sensitized with gold salts.

16. The emulsion of claim 9 which is additionally chemically sensitized with gold salts.

17. The emulsion of claim 10 which is additionally chemically sensitized with gold salts.
18. The emulsion of claim 14 which is additionally chemically sensitized with gold salts.
19. The emulsion of claim 1 which is additionally chemically sensitized with reduction sensitizers. 5
20. The emulsion of claim 8 which is additionally chemically sensitized with reduction sensitizers.
21. The emulsion of claim 10 which is additionally chemically sensitized with reduction sensitizers. 10
22. The emulsion of claim 8 which is additionally chemically sensitized with gold salts and reduction sensitizers.
23. The emulsion of claim 11 which is additionally chemically sensitized with gold salts and reduction sensitizers. 15
24. The emulsion of claim 12 which is additionally chemically sensitized with gold salts and reduction sensitizers.

## References Cited in the file of this patent

## UNITED STATES PATENTS

|           |                      |               |
|-----------|----------------------|---------------|
| 1,738,530 | Frankenburger et al. | Dec. 10, 1929 |
| 2,059,642 | Kankelwitz           | Nov. 3, 1936  |
| 2,240,472 | Swan                 | Apr. 29, 1941 |
| 2,400,532 | Blake et al.         | May 21, 1946  |
| 2,423,549 | Blake                | July 8, 1947  |
| 2,441,389 | Blake                | May 11, 1948  |
| 2,487,850 | Carroll              | Nov. 15, 1949 |
| 2,540,086 | Baldsiefen           | Feb. 6, 1951  |

## FOREIGN PATENTS

|         |               |               |
|---------|---------------|---------------|
| 633,159 | Great Britain | Dec. 12, 1949 |
|---------|---------------|---------------|